

June 3, 1924.

1,496,607

H. F. SAUNDERS

PROCESS FOR PRODUCING FERRIC OXIDE

Filed Aug. 3, 1922



Inventor  
Harold F. Saunders  
*J. F. Edwards*  
Attorney

## UNITED STATES PATENT OFFICE.

HAROLD F. SAUNDERS, OF CLEVELAND, OHIO, ASSIGNOR TO THE CHEMICAL SPECIALTIES COMPANY, OF CLEVELAND, OHIO, A CORPORATION OF OHIO.

## PROCESS FOR PRODUCING FERRIC OXIDE.

Application filed August 3, 1922. Serial No. 579,360.

To all whom it may concern:

Be it known that I, HAROLD F. SAUNDERS, a citizen of the United States, residing in the city of Cleveland, county of Cuyahoga, and State of Ohio, have invented certain new and useful Improvements in Processes for Producing Ferric Oxide, of which the following is a specification.

This invention relates to the manufacture of ferric oxide by an electrolytic process.

The principal aims of my invention are to provide a process for producing, quickly and cheaply, ferric oxides having extreme fineness of particle, and which are particularly valuable as pigments, and having increased covering power.

When an electrolyte composed of an ionizable salt in solution is electrolyzed by a direct current in a cell consisting of an iron anode and a cathode of any conducting material, and the products of the reaction, consisting principally of ferrous hydroxide, are exposed to the air, there is a gradual oxidation to form both ferric and ferroso-ferric oxide, the latter in considerable proportion. The ferroso-ferric oxide being relatively the more stable, it is difficult to obtain a pure ferric oxide by this means.

The oxides of iron obtained by electrolytic means possess certain physical characteristics, such as extreme fineness of particle, which render them particularly valuable as pigments owing to the increased covering power obtained.

I have found that when an oxidizing agent such as air is so completely diffused in the electrolytic bath as to be in contact with all the reacting agents, the product obtained consists entirely of ferric oxide, and retains all the desirable physical characteristics of the electrolytic oxides.

In order that a clearer understanding of my invention may be had, attention is hereby directed to the accompanying drawing illustrating, diagrammatically, one possible form of apparatus whereby my process may be carried out, the container being shown in vertical section.

Referring to the drawing and as an example of my process, in a suitable container 1, there is placed a bath 2, which is composed of an ionizable salt in solution, and in which is placed a plate of iron 3 to serve as the anode, and a second plate 4 of any conducting material to serve as the cathode. At the

bottom of the bath is placed a coil 5 of perforated pipe connected to a suitable source of air supply, such as tank 6, and through the perforations 7 air is caused to bubble up in the form of fine bubbles 8, so as to permeate the whole bath and be intimately diffused over the entire reacting surfaces. When a direct current of electricity, as from battery 9, is passed through the bath from anode to cathode, reaction takes place with the direct formation of ferric oxide according to the following equations, assuming the use of sodium sulphate as the salt in the electrolyte:



The sodium sulphate is electrolyzed to sodium hydroxide and sulphuric acid. The sulphuric acid dissolves the iron at the anode forming sulphate of iron, and this sulphate of iron combines with the sodium hydroxide formed at the anode and oxygen from the introduced air with the direct formation of ferric oxide.

The sodium sulphate is thus regenerated and is separated from the ferric oxide by filtration and returned to the bath, thus rendering the process continuous. The ferric oxide is dried and appears as a reddish brown powder which is seen under the microscope to be in an extremely fine state of division, practically approaching colloidal condition. It is this fineness which gives to the product its intensity of covering power. This product is a pigment of exceptionally high quality and commercial value. 90 95

Since many different salts may be used in the electrolyte and since many different forms of iron may be used as anodic material, and as many other changes in operation may be employed without departing from the scope of my invention, it is intended that all matter contained in the above description or illustrated in the accompanying drawing shall be interpreted as illustrative and not in a limiting sense. 100 105

What I claim is:

1. The process of producing ferric oxide, which consists of electrolyzing an ionizable salt solution in the presence of an iron anode and an oxidizing agent. 110

2. The process of producing ferric oxide, which consists of electrolyzing an ionizable salt solution in the presence of an iron anode and air.
3. The process of producing ferric oxide, which consists of acting upon iron in the presence of air with the products of electrolysis of the solution of an ionizable salt.
4. The process of producing ferric oxide, which consists of electrolyzing sodium sulphate in solution in the presence of an iron anode and an oxidizing agent.
5. The process of producing ferric oxide, which consists of providing an electrolyte, consisting of an ionizable salt solution, providing an iron anode and a conducting cathode in said electrolyte, and simultaneously establishing electrolysis, and permeating the bath with an oxidizing agent.
6. The process of producing a ferric pigment, which consists of producing hydrated ferric oxide in an electrolytic bath, removing the hydrated ferric oxide so produced from said bath and drying said oxide.
7. The process of producing hydrated

ferric oxide, which consists of electrolyzing sodium sulphate in solution in the presence of an iron anode and simultaneously conducting air into the bath so as to diffuse over the reacting surfaces.

8. The process of producing ferric oxide, which consists of oxidizing ferrous hydrate with air at the point and time of formation in an electrolytic bath, and removing said hydrate from the bath and drying.

9. The process of producing ferric oxide, which consists in passing an electric current between an iron anode and a cathode of any conducting material, suspended in a bath consisting of an aqueous solution of an ionizable salt, to precipitate out ferrous hydrate, and intimately diffusing air throughout said bath to oxidize the ferrous hydrate to ferric hydrate at the point and time of formation, removing said hydrate from the bath and drying.

This specification signed this 28th day of July, 1922.

HAROLD F. SAUNDERS.